

Dec. 24, 1963

F. G. CIAPETTA ET AL.

3,115,456

## METHOD FOR INITIATING CYCLE OPERATION

Filed July 6, 1959



*Inventors  
Frank G. Ciapetta  
Harry L. Coonradt  
William E. Garwood*

By Andrew J. Gabrini, Jr.  
Attorney

1

3,115,456

**METHOD FOR INITIATING CYCLE OPERATION**  
Frank G. Ciapetta, Silver Spring, Md., and Harry L. Coonradt, Woodbury, and William E. Garwood, Haddonfield, N.J., assignors to Socony Mobil Oil Company, Inc., a corporation of New YorkFiled July 6, 1959, Ser. No. 825,183  
6 Claims. (Cl. 208—111)

This application is a continuation-in-part of copending application Serial Number 551,701, filed December 7, 1955, now abandoned.

This invention relates to catalytic cracking. It is more particularly concerned with the initiation of cycle operation of a cracking process that is carried out in the presence of hydrogen.

In copending application Serial Number 813,247, filed May 14, 1959, which is a continuation-in-party of Serial Number 491,256, filed March 1, 1955, now abandoned, a cracking process is described that involves contacting a blend of virgin stock and cycle stock with a platinum or palladium-containing catalyst in the presence of hydrogen at superatmospheric pressures. This operation, as compared with a once-through operation with the virgin stock alone, offers many advantages, including lower temperature, lower dry gas yield, lower light naphtha yield, greater heavy naphtha yield, and a fuel oil having a higher diesel index. These advantages are especially pronounced in the case of heavy charge stocks, such as heavy gas oils, vacuum gas oils, topped crude, etc., as these charge stocks require relatively severe cracking conditions in a once-through operation. Recycle operation results in greater catalyst stability during long runs. Thus, in a once-through operation using heavy gas oil, the catalyst loses activity at the rate of about 3° F. per day. On the other hand, in cycle operation this loss in activity is reduced to less than 1° F. per day.

Ordinarily, sufficient cycle stock derived from the heavy stocks will not be available to initiate a recycle operation. To be sure, cycle stock can be obtained by cracking the heavy charge stock in a once-through operation until sufficient is produced. This manner of operation, however, is disadvantageous to over-all refinery operation, because the relatively large yields of dry gas and light naphtha decrease the total useful output.

It has now been found that cycle operation for cracking heavy stocks can be initiated by a method that is simple and economical. It has been discovered that the cycle operation of a cracking process carried out in the presence of a platinum- or palladium-containing catalyst and of hydrogen can be initiated by first cracking a blend of the heavy charge stock with a light gas oil until sufficient cycle stock is available, and then discontinuing the use of light gas oil and carrying out the desired recycle operation.

Accordingly, it is an object of this invention to provide a method for initiating a recycle cracking operation. Another object is to provide a method for initiating a process that involves cracking a mixture of a heavy charge stock and cycle stock. A specific object is to provide a method for initiating a process that involves cracking a mixture of a heavy charge stock and cycle stock in contact with a platinum- or palladium-containing catalyst and in the presence of hydrogen. Another specific object is to provide a method for obtaining sufficient cycle stock to commence the cycle cracking of a heavy charge stock that is simple and economical, and which does not involve once-through cracking of the heavy charge stock.

Other objects and advantages of the process of this invention will become apparent to those skilled in the art from the following detailed description considered in conjunction with the drawings, wherein

2

FIGURE 1 presents a diagrammatic representation of the process of this invention;

FIGURE 2 presents the graphic relationship between the volume percent conversion into products boiling at temperatures lower than about 390° F. and the temperature for cracking a typical heavy gas oil, a typical mixture of heavy gas oil with light gas oil, a typical mixture of heavy gas oil with cycle stock obtained by cracking a mixture of heavy gas oil with light gas oil, and a typical mixture of heavy gas oil with cycle stock obtained by cracking the heavy gas oil.

The present invention provides, in a recycle cracking process wherein a mixture of a heavy gas oil with cycle stock obtained from cracking said heavy gas oil and in which the volumetric ratio of said cycle stock to said heavy gas oil varies between about 0.1:1, respectively, and about 10:1, respectively, is contacted with a catalyst comprising between about 0.05 percent and about 20 percent, by weight of the catalyst, of at least one metal of the platinum and palladium series deposited upon a synthetic composite of the solid oxides of at least two elements of groups II A, II B, and IV of the periodic arrangement of the elements, having an activity index of at least 25, in the presence of hydrogen in amounts, expressed in molar ratio of hydrogen to hydrocarbon charge, within the range about 2 to about 80, at pressures about 100 pounds per square inch gauge, at a liquid hourly space velocity within the range about 0.1 to about 10, and at a temperature above about 500° F., the method of initiating said recycle cracking process that comprises initially contacting with said catalyst a mixture of a light gas oil with said heavy gas oil in which the volumetric ratio of said light gas oil to said heavy gas oil is within the range about 10:1, respectively, and about 0.1:1, respectively, in the presence of hydrogen and under substantially the same conditions of hydrogen to hydrocarbon molar ratio, pressure, space velocity, and temperature that are employed in said recycle cracking process, continuing to charge said mixture for a period of time to produce sufficient cycle stock for said recycle cracking process, and subsequently replacing said light gas oil in said mixture of light gas oil and heavy gas oil with said cycle stock.

A method of operating the process of this invention is illustrated in FIGURE 1. A light charge stock is introduced through a pipe 10 and pumped by means of a metering pump 11 through pipes 12 and 13 into a furnace, or other suitable heating means, 14. The heavy charge stock to be cracked is introduced through a pipe 15 and is pumped by means of a metering pump 16 through pipes 17 and 18 and introduced into the furnace 14 in admixture with the light charge stock.

The mixture of light and heavy charge stock is heated in the furnace 14 to the desired conversion temperature. The thus-heated mixture is passed through pipes 19 and 20 into a reactor 20.

Hydrogen gas, or a gas rich in hydrogen, is introduced through a pipe 21 and compressed by means of a compressor 22 to the desired reaction pressure. The compressed hydrogen is then passed through a pipe 23 into a heat exchanger 24 wherein it is heated to reaction temperature. The heated hydrogen is then passed through pipe 19 in admixture with the hydrocarbon charge into the reactor 20. Alternatively, the mixture of hydrogen and charge stocks can be heated together in a common heater.

The reactor 20 contains a static bed of a platinum or palladium series metal catalyst. Suitable catalysts are described in copending application Serial Number 418,166, filed March 23, 1954. The mixture of hydrocarbons and hydrogen gas are contacted with the catalyst at a liquid hourly space velocity and temperature suffi-

cient to effect the desired amount of conversion. In order to produce sufficient cycle stock (products boiling at temperatures higher than about 390° F.), it is generally preferred to operate the process so that there is effected no more than 50 volume percent conversion into products boiling at temperatures lower than about 390° F. In general, the amount of conversion into products boiling at temperatures lower than about 390° F. will be between about 10 and about 50 volume percent. The total effluent from the reactor 20 is removed through a pipe 25 and passed through a heat exchanger 26 wherein the products are cooled to temperatures at which hydrogen can be separated. The thus-cooled product is passed through a pipe 27 into a high pressure gas separator 28.

In the gas separator 28, a gas rich in hydrogen is separated from the liquid product. The hydrogen-containing gas is removed from the high pressure separator 28 through a pipe 29 and recycled to the process via pipe 23. In pipe 23 the recycle hydrogen gas is admixed with sufficient fresh hydrogen to maintain the desired hydrogen to oil molar ratio in the process.

The liquid product from the separator 28 is removed through a pipe 30 and passed through a depressuring zone 31 and a pipe 32 into a fractionator 33. In the fractionator 33 the reaction products are separated into suitable fractions. Ordinarily, the dry gas is removed through a pipe 34. Butanes are removed through a pipe 35 and light and heavy naphtha fractions are removed through pipes 36 and 37, respectively. The product boiling at temperatures higher than about 390° F. is removed from the fractionator 33 through a pipe 38 and passed into a suitable storage vessel 39.

When sufficient cycle stock has been obtained in the storage vessel 39 to initiate recycle operation with a heavy charge stock alone, cycle stock is removed from the storage vessel through a pipe 40. Then, the cycle stock is pumped through a metering pump 41 through a pipe 42 into pipe 13 in an amount sufficient to effect the desired ratio of recycle to heavy charge stock. At the same time, the flow of light charge stock is discontinued. This operation is effected by suitable manipulation of valves 43 and 44. From this point on, the process then operates as a straight recycle process.

In an alternative method of operating the process, the storage vessel 39 can be eliminated. Then, the recycle stock as it becomes available is pumped directly into pipe 13. As more and more cycle stock becomes available, the amount of light charge stock is reduced accordingly by suitable control of valve 44 and of metering pump 11. When sufficient cycle stock is being produced to maintain the recycle operation, the flow of light charge stock is discontinued entirely and the straight recycle process continues.

Throughout the specification and the claims, the term "conversion" is intended to be a generic term for the amount of products boiling at temperatures lower than about 390° F. (100-recycle), of gasoline, or of fuel oil obtained in the process. It is expressed in terms of the volume percent of the initial charge which is transformed in the process. The amount of product boiling at temperatures lower than about 390° F. is obtained by subtracting the volume percent of cycle stock from 100 percent, i.e., from the initial volume of the charge. The expression "(100-recycle)" is an abbreviation for 100 percent minus the volume percent recycle. "Dry gas" refers to the methane, ethane, propane, and ethylene and propylene produced in a cracking process, expressed in terms of weight percent of the initial charge. "Light naphtha" is the product that boils between about 125° F. and about 170° F. The "heavy naphtha" is the product that boils between about 170° F. and about 390° F. The "diesel index" of the fuel oil is a function of the A.P.I. gravity and the aniline number, as defined by Becker et al. in the S.A.E. Journal (Transactions), vol. 35, No. 4, p. 377. The cracking activity of a carrier is expressed in terms

of the percent, by volume, of a standard hydrocarbon charge which is cracked, under specific operating conditions, in the "Cat. A" test. This test is described by Alexander and Shimp in National Petroleum News, 36, page R-537 (August 2, 1944). The unit for rating the cracking activity of a material is called the "activity index" (A.I.).

The catalysts utilizable herein are those described in U.S. 2,945,806, issued July 19, 1960. Briefly, these catalysts comprise between about 0.05 percent, by weight, and about 20 percent, by weight of the final catalyst, preferably between about 0.1 percent and about 5 percent, by weight, of the metals of the platinum and palladium series, i.e., those having atomic numbers of 44-46, inclusive, 76-78, inclusive, supported upon synthetic composites of two or more refractory oxides. The carrier is a synthetic composite of two or more solid oxides of the elements of groups IIA, IIIB and IVA and B of the periodic arrangement of elements [J. Chem. Ed., 16, 409 (1939)]. These synthetic composites of refractory oxides must have an activity index of at least about 25. They can also contain halogens and other materials which are known in the art as promoters for cracking catalysts, or small amounts of alkali metals that are added for the purpose of controlling the activity index of the carrier. Non-limiting examples of the composites contemplated herein include silica-alumina, silica-zirconia, silica-alumina-zirconia, silica-alumina-thoria, alumina-boria, silica-magnesia, silica-alumina-magnesia, silica-alumina-fluorine, and the like. The preferred support is a synthetic composite of silica and alumina containing between about 1 percent, by weight, and about 90 percent, by weight, of alumina. These synthetic composites of two or more refractory oxides can be made by any of the usual methods known to those skilled in the art of catalyst manufacture. Examples of methods of preparing them are set forth in U.S. 2,945,806, issued July 19, 1960.

The following example illustrates a method of preparing a platinum-containing catalyst utilizable in the process of this invention:

#### EXAMPLE 1

A synthetic silica-alumina carrier or support containing 10 percent by weight alumina was prepared by mixing an aqueous solution of sodium silicate (containing 158 g. per liter of silica) with an equal amount of an aqueous acid solution of aluminum sulfate containing 39.4 g.  $\text{Al}_2(\text{SO}_4)_3$  and 28.6 g. concentrated  $\text{H}_2\text{SO}_4$  per liter. This mixture of solutions was dropped through a column of oil, wherein gelation of the hydrogel was effected in bead form. The bead hydrogel was soaked in hot water (about 120° F.) for about 3 hours. The sodium in the hydrogel was then removed by exchanging the gel with an aqueous solution of aluminum sulfate [1.5%  $\text{Al}_2(\text{SO}_4)_3$  by weight] containing a small amount (0.2 percent by weight) of ammonium sulfate. The thus-exchanged hydrogel bead was water-washed. Then, it was dried in superheated steam (about 280-340° F.) for about 3 hours and, finally, calcined at 1300° F. under a low partial pressure of steam for about 10 hours.

The silica-alumina beads were then crushed to pass through a 14-mesh screen and the material retained on a 25-mesh screen (U.S. Standard Screen Series) was used for catalyst preparation. Portions of the crushed, calcined carrier were then barely covered with aqueous solutions of chloroplatinic acid, of concentrations sufficient to produce the desired amount of metal in the finished catalyst. The excess solution was removed by centrifuging. The thus-impregnated carrier was then dried at 230° F. for 24 hours. The catalyst was treated with hydrogen for 2 hours at 450° F. Then, it was activated in hydrogen for 2 hours at 900° F. before it was used. The catalyst thus-prepared contained 0.47 percent platinum, by weight of the catalyst. Its silica-alumina carrier had an activity index of 46.

The light charge stock that is charged to the process of this invention is a hydrocarbon fraction that has an initial boiling point of about 390-400° F. and an end boiling point of about 600-650° F. The heavy charge stock is a hydrocarbon fraction that boils within the range varying between about 400° F. and about 1200° F. and higher. This material can be a heavy gas oil, a heavy fraction obtained by destructive hydrogenation of coals, tars, pitches, etc., a vacuum gas oil, mixtures of medium and heavy gas oils, topped deasphalted crudes, and the like. Both the light and heavy charge materials can be gas oils, refractory cycle stocks from conventional cracking, hydrocarbon fractions obtained by destructive distillation of coal, tars, pitches, asphalts, etc.

The light charge stock that is admixed with the heavy charge stock can be from the same source as the heavy charge stock, or it can be from a different source. The relative amounts of light and heavy stocks are adjusted so that the reaction conditions for cracking the mixture will substantially be the same as the reaction conditions ultimately to be used in cracking the heavy charge stock in a recycle operation. Generally, the volume ratio of light charge stock to heavy charge stock will be within the range about 10:1, respectively, to about 0.1:1, respectively, preferably between about 5:1, respectively, and 1:1, respectively.

The presence of even relatively small amounts of nitrogen compounds in the charge stock causes the degree of conversion that can be attained at any given temperature to decrease. Thus, the higher the nitrogen content the greater will be the temperature needed to effect a given amount of conversion. Since higher temperatures are usually associated with higher dry gas production, there will usually be a greater quantity of dry gas produced when converting high nitrogen stocks to the same degree as lower nitrogen stocks.

It is, therefore, preferred for optimum operations that the cracking charge stocks contain less than about 0.1 percent nitrogen, by weight, and still more preferably less than about 0.08 percent, by weight.

If desired, the nitrogen content of a charge stock may be reduced to an amount less than about 0.1 weight percent, and, preferably, below about 0.08 weight percent, before charging to the process of this invention by any of the methods well-known in the art, such as, for example, acid treatment, propane deasphalting, and hydrogenolysis under very high pressure, in contact with catalysts such as molybdenum or tungsten oxide, nickel sulfide, tungsten sulfide, cobalt molybdate, cobalt tungstate, etc.

In order to obtain the best results in the recycle cracking process that is initiated by the method of this invention, the ratio of cycle stock to virgin stock (charge stock that has not been subjected to the process of this invention or to processes described in the aforementioned pending applications) in the charge ordinarily should be at least about 0.1:1. The ratio of cycle stock to virgin stock can be as high as 15:1 or higher. In practice, however, it is preferred to use cycle stock to virgin stock, volume ratios within the range about 0.1:1 to about 10:1 and higher and more preferably within the range about 1:1 to about 5:1.

As has been mentioned hereinbefore the initiation process of this invention is carried out under substantially the same conditions as the final cracking process. Thus, conditions of hydrogen pressure, hydrogen-to-oil molar ratio, and space velocity will usually be the same. Throughout the initiation process and the ultimate cracking process, the temperature might be somewhat different. However, a volume ratio of light charge stock to heavy charge stock is selected so that the curve defining the relationship between the temperature and the volume percent conversion into products boiling at temperatures lower than about 390° F. will be substantially identical with the curve defining this relationship in the ultimate cycle cracking process.

In so far as is known, there is nothing critical about the reaction temperature at which the process of this invention is carried out, and it is believed operable at any temperatures, conventional in the art, at which hydrocracking, with a net consumption of hydrogen by the charge stock, will occur. Of course, the reaction temperature should not generally exceed the minimum temperature at which the charge is converted completely into products boiling below 390° F. or some other end point that is more desirable. For the reaction to proceed at an acceptable rate, it is usually necessary that the reaction temperature exceed about 500° F. Preferably, the reaction temperature should be within the range about 500° F. to about 825° F., and still more preferably within the range 650° F. to 825° F.

Likewise, in so far as is known, there is nothing critical about the reaction pressure employed in this invention and it will operate at any hydrogen pressures, conventional in the art, which effect hydrocracking with a net consumption of hydrogen by the charge stocks. Very high pressures, however, make it necessary to employ very expensive, heavy-walled reactors. It is, therefore, preferable that the hydrogen pressure be within the range 100 to 2500 pounds per square inch gauge (p.s.i.g.). The liquid hourly space velocity should be within the range about 0.1 to about 10, preferably between about 0.1 and about 4 volumes of reactant (as 60° F. liquid) per volume of catalyst per hour. The molar ratio of hydrogen to hydrocarbon should be within the range about 2 to about 80, preferably between about 5 and about 50.

The cracking process can be carried out using conventional apparatus and schemes for effecting recycle operation in catalytic cracking. As the catalyst remains active over long periods of time before it must be regenerated, the operation is advantageously carried out using a fixed bed of catalyst. Other techniques, however, can be used, such as the moving bed technique or the fluid bed technique.

#### EXAMPLE 2

The charge stock used in this run was a mixture containing 57.7 volume percent of light gas oil and 42.3 volume percent heavy gas oil distilled from Kuwait crude. Pertinent properties of these Kuwait gas oils and of this mixture are as follows:

|                                           | Light<br>Gas<br>Oil | Heavy<br>Gas<br>Oil | Gas<br>Oil<br>Blend |
|-------------------------------------------|---------------------|---------------------|---------------------|
| A.P.I. Gravity                            | 39.1                | 27.6                | 33.8                |
| Distillation, Vacuum Assay <sup>1</sup> : |                     |                     |                     |
| I.B.P.                                    | 418                 |                     |                     |
| 5%                                        |                     | 648                 | 467                 |
| 50%                                       | 506                 | 724                 | 590                 |
| 95%                                       |                     | 814                 | 787                 |
| E.P.                                      | 634                 |                     | 787                 |
| Sulfur, Weight Percent                    | 0.94                | 2.06                | 1.51                |

<sup>1</sup> Distillation data for light gas oil are A.S.T.M. distillation.

The blend of light and heavy gas oil was subjected to cracking in the presence of hydrogen and of the catalyst described in Example 1, after the latter had reached equilibrium, i.e., had been in continuous operation for more than 5 days. The hydrogen pressure used was 1000 p.s.i.g., the liquid hourly space velocity was 0.5 and the molar ratio of hydrogen-to-oil was 40. The cracking was carried out at a temperature of about 730° F. There was effected 56.7 volume percent conversion into products boiling below about 390° F. The gaseous products were separated from the liquid products. Then, the liquid products were subjected to fractionation. The pertinent results of this run are set forth in Table I.

#### EXAMPLE 3

The charge used in this example was a mixture of 1 volume of cycle stock produced in the run described in Example 2 and 1 volume of the heavy Kuwait gas oil that

was defined in Example 2. The cycle stock and the blend of cycle stock and heavy gas oil had the following properties:

|                                           | Cycle Stock | Blend |
|-------------------------------------------|-------------|-------|
| A.P.I. Gravity                            | 43.6        | 35.3  |
| Distillation, Vacuum Assay <sup>1</sup> : |             |       |
| I.B.P.                                    | 416         |       |
| 5%                                        | 458         |       |
| 50%                                       | 472         | 636   |
| 95%                                       | 500         | 798   |
| E.P.                                      | 624         |       |
| Sulfur, Weight Percent                    | 0.11        | 1.08  |

<sup>1</sup> Distillation data for the cycle stock are A.S.T.M. distillation data.

This blend was subjected to cracking in the presence of hydrogen and of the catalyst described in Example 1, after the latter had reached equilibrium. The hydrogen pressure used was 1000 p.s.i.g., the liquid hourly space velocity was 0.5 and the molar ratio of hydrogen-to-oil was 40. The cracking was carried out at a temperature of about 700° F. whereby there was effected a conversion of about 40.5 volume percent into products boiling lower than about 390° F. Separation between the gaseous products and the liquid products was effected and the

stock and the blend of cycle stock and heavy gas oil had the following properties:

|                                           | Cycle Stock | Blend |
|-------------------------------------------|-------------|-------|
| A.P.I. Gravity                            | 36.0        | 31.7  |
| Distillation, Vacuum Assay <sup>1</sup> : |             |       |
| I.B.P.                                    | 420         |       |
| 5%                                        | 464         |       |
| 50%                                       | 570         | 684   |
| 95%                                       | 698         | 796   |
| E.P.                                      | 698         |       |
| Sulfur, Weight Percent                    | 0.20        | 1.00  |

<sup>1</sup> Distillation data for the cycle stock are A.S.T.M. distillation data.

This blend was subjected to cracking in the presence of hydrogen and the catalyst described in Example 1, after the latter had reached equilibrium. The hydrogen pressure used was 1000 p.s.i.g., the liquid hourly space velocity was 0.5 and the molar ratio of hydrogen-to-oil was 40. Cracking was carried out at a temperature of about 710° F., whereby there was effected a conversion of about 36.9 volume percent into products boiling below about 390° F. The gaseous and liquid products were separated and the liquid product was fractionated. Pertinent results are set forth in Table I.

Table I

| Charge                                | Mixture of Light and Heavy Gas Oil | Mixture of Cycle Stock and Heavy Gas Oil | Heavy Kuwait Gas Oil |       |       | Mixture Cycle (4) and Heavy Gas Oil |
|---------------------------------------|------------------------------------|------------------------------------------|----------------------|-------|-------|-------------------------------------|
| Example No.                           | 2                                  | 3                                        | 4                    | 4     | 4     | 5                                   |
| Conditions:                           |                                    |                                          |                      |       |       |                                     |
| Temp., ° F.                           | 730                                | 700                                      | 743                  | 793   | 785   | 710                                 |
| Pressure, P.s.i.g.                    | 1,000                              | 1,000                                    | 1,000                | 1,000 | 1,100 | 1,000                               |
| LHSV                                  | 0.5                                | 0.5                                      | 0.5                  | 0.5   | 0.5   | 0.5                                 |
| H <sub>2</sub> /oil molar ratio       | 40                                 | 40                                       | 40                   | 40    | 40    | 40                                  |
| Results:                              |                                    |                                          |                      |       |       |                                     |
| Conversion, Vol. Percent <sup>1</sup> | 56.7                               | 40.5                                     | 28.1                 | 69.2  | 52.4  | 46.9                                |
| Dry Gas, Wt. Percent                  | 2.1                                | 1.9                                      | 2.2                  | 5.9   | 3.8   | 1.8                                 |
| Butanes, Vol. Percent                 | 7.6                                | 5.5                                      | 4.8                  | 14.8  | 11.6  | 8.8                                 |
| Pentanes, Vol. Percent                | 7.6                                | 5.1                                      | 4.3                  | 11.9  | 9.1   | 6.9                                 |
| Lt. Naphtha, Vol. Percent             | 5.6                                | 2.6                                      | 3.7                  | 9.7   | 7.6   | 4.8                                 |
| Hvy. Naphtha, Vol. Percent            | 46.2                               | 34.3                                     | 23.6                 | 42.4  | 36.3  | 37.2                                |
| Fuel Oil, Vol. Percent                | 43.3                               | 59.5                                     | 71.9                 | 30.8  | 47.6  | 53.1                                |
| Diesel Index of Fuel Oil              | 73.7                               | 73.6                                     | 64.4                 | 71.0  | 58.9  | 68.8                                |

<sup>1</sup> Conversion into products boiling at temperatures lower than about 390° F.

liquid product was fractionated. Pertinent results are set forth in Table I.

#### EXAMPLE 4

The charge stock used in this run was the heavy Kuwait gas oil that was defined in Example 2. This gas oil alone was subjected to cracking in the presence of hydrogen and of the catalyst described in Example 1 after the latter had reached equilibrium. The hydrogen pressure used was 1000 p.s.i.g., the liquid hourly space velocity was 0.5 and the molar ratio of hydrogen-to-oil was 40. Cracking was carried out in three runs. Each run was effected at a different temperature, namely about 743° F., about 793° F. and about 785° F. The products of each run were separated into gaseous and liquid products and the liquid products were fractionated. Pertinent results are set forth in Table I.

#### EXAMPLE 5

The charge stock used in this run was a mixture of 1 volume of the heavy Kuwait gas oil described in Example 2 and 1 volume of the cycle stock obtained by cracking the heavy Kuwait gas oil at a temperature of about 785° F., as described in Example 4. The cycle

The run described in Example 2, using the mixture of light and heavy gas oil, illustrates the initial stages of the initiating process of this invention. As described hereinbefore, this operation is continued until sufficient cycle stock is obtained to use a cycle operation. At that time, the charging of the light gas oil is discontinued (either suddenly, or gradually, as described hereinbefore) and the operation is continued using a charge composed of cycle stock and the heavy gas oil. This operation is illustrated in Example 3. Ultimately, of course, the cycle stock obtained by cracking the mixture of light and heavy gas oils that was used to initiate the cycle operation will become extinct. At that time the operation will involve a recycle operation wherein the recycle stock is obtained by cracking the heavy gas oil. This ultimate stage of the operation is illustrated by the run described in Example 5.

The curves set forth in FIGURE 2 are based upon the data in Table I. Curve A shows the graphic relationship between temperature and the volume percent conversion of the charge into products boiling at temperatures lower than 390° F., when cracking under substantially identical conditions, the mixture of light and heavy gas oils; the mixture of heavy gas oil and cycle stock obtained from cracking the mixture of light and

heavy gas oil; and the mixture of heavy gas oil and cycle stock obtained from cracking the heavy gas oil. It will be noted that the volume percent conversion-temperature relationship for all these operations falls upon a common curve. Thus, for example, the blend of 57.7 volume percent of light gas oil and 43.7 volume percent heavy gas oil cracks in the same temperature-conversion relationship as does the ultimate recycle operation using the heavy gas oil plus cycle stock therefrom in a 1:1 volume ratio. In other words, if the temperature of the ultimate operation, such as is described in Example 5 were elevated to 730° F. as used in the initiating run, there would be obtained a conversion of about 56 volume percent into products boiling at temperatures lower than about 390° F.

Curve B defines the relationship between the temperature and the volume percent conversion into products boiling at temperatures lower than about 390° F. obtained when cracking the heavy Kuwait gas oil. This curve is included for purposes of comparison. It will be noted that the initiating process and the ultimate recycle operation described herein are all effected at temperatures substantially lower than those required for cracking the heavy gas oil alone. It has been found that the relationship between the volume percent conversion and (1) the weight percent dry gas, (2) the volume percent light naphtha and (3) the volume percent heavy naphtha will define a common curve, as was experienced in the case of curve A in FIGURE 2. A comparison of these curves with corresponding curves obtained by cracking the heavy gas oil alone shows that there is achieved all the advantageous results described hereinbefore, namely lower dry gas yield, lower light naphtha yield and a higher yield of heavy naphtha.

Another advantage of this invention may be noted. With catalysts of the type described herein there is an initial period of operation, when the catalyst is fresh, in which the catalyst performs in a quite different manner from its typical performance after some aging has occurred. Use of a heavy gas oil charge during this period has been found substantially less desirable than use of a light gas oil because the heavy gas oil has, on occasion, damaged specific catalyst functions. The use of a blend of light and heavy gas oils during the start-up period in this invention insures that this damage does not occur.

Although the present invention has been described with preferred embodiments, it is to be understood that modifications and variations may be resorted to, without departing from the spirit and scope of this invention, as those skilled in the art will readily understand. Such variations and modifications are considered to be within the purview and scope of the appended claims.

We claim:

1. In a recycle cracking process wherein a mixture of a heavy hydrocarbon charge stock with cycle stock boiling above about 390° F. obtained from hydrocracking said heavy hydrocarbon charge stock and in which the volumetric ratio of said cycle stock to said heavy hydrocarbon charge stock varies between about 1:1, respectively, and about 10:1, respectively, is contacted with a catalyst comprising between about 0.05 percent and about 20 percent, by weight of the catalyst, of at least one metal of the platinum and palladium series of metals deposited upon a synthetic composite of the solid oxides of at least two elements of groups IIA, IIIB and IV of the periodic arrangement of the elements, said composite having an activity index of at least 25, in the presence of hydrogen in amounts, expressed in molar ratio of hydrogen to hydrocarbon charge, varying between about 2 and about 80, at pressures varying between about 100 pounds per square inch gauge and about 2500 pounds per square inch gauge, at a liquid hourly space velocity varying between about 0.1 and about 10, and at temperatures varying between about 500° F. and about 825° F.; the

method of initiating said recycle cracking process that comprises initially contacting with said catalyst a mixture of a light hydrocarbon charge stock boiling within the range of about 390° F. to 650° F. with said heavy hydrocarbon charge stock, in which the volumetric ratio of said light hydrocarbon charge stock to said heavy hydrocarbon charge stock varies between about 1:1, respectively, and about 10:1, respectively, in the presence of hydrogen, and under substantially the same conditions of hydrogen to hydrocarbon molar ratio, pressure, space velocity and temperature that are employed in said recycle cracking process, continuing to charge said mixture for a period of time to produce sufficient cycle stock for said recycle cracking process, and subsequently replacing said light hydrocarbon charge stock in said mixture of light hydrocarbon charge stock and heavy hydrocarbon charge stock with said cycle stock.

2. In a recycle cracking process wherein a mixture of a heavy gas oil boiling within the range varying between about 400° F. and about 1200° F. with cycle stock boiling above about 390° F. obtained from hydrocracking said heavy gas oil and in which the volumetric ratio of said cycle stock to said heavy gas oil varies between about 1:1, respectively, and about 10:1, respectively, is contacted with a catalyst comprising between about 0.05 percent and about 20 percent, by weight of the catalyst, of at least one metal of the platinum and palladium series of metals deposited upon a synthetic composite of the solid oxides of at least two elements of groups IIA, IIIB and IV of the periodic arrangement of the elements, said composite having an activity index of at least 25, in the presence of hydrogen in amounts, expressed in molar ratio of hydrogen to hydrocarbon charge, varying between about 2 and about 80, at pressures varying between about 100 pounds per square inch gauge and about 2500 pounds per square inch gauge, at a liquid hourly space velocity varying between about 0.1 and about 10, and at temperatures varying between about 500° F. and about 825° F., the method of initiating said recycle cracking process that comprises initially contacting with said catalyst a mixture of a light gas oil boiling within the range varying between about 390-400° F. and about 600-650° F. with said heavy gas oil in which the volumetric ratio of said light gas oil to said heavy gas oil varies between about 1:1, respectively, and about 10:1, respectively, in the presence of hydrogen, and under substantially the same conditions of hydrogen to hydrocarbon molar ratio, pressure, space velocity and temperature that are employed in said recycle cracking process, continuing to charge said mixture for a period of time to produce sufficient cycle stock for said recycle cracking process and subsequently replacing said light gas oil in said mixture of light gas oil and heavy gas oil with said cycle stock.

3. In a recycle cracking process wherein a mixture of a heavy gas oil boiling within the range varying between about 400° F. and about 1200° F. with cycle stock boiling above about 390° F. obtained from hydrocracking said heavy gas oil and in which the volumetric ratio of said cycle stock to said heavy gas oil varies between about 1:1, respectively, and about 5:1, respectively, is contacted with a catalyst comprising between about 0.1 percent and about 5 percent, by weight of the catalyst, of platinum deposited upon a synthetic composite of silica and alumina, said composite having an activity index of at least 25, in the presence of hydrogen in amounts, expressed in molar ratio of hydrogen to hydrocarbon charge, varying between about 5 and about 50, at pressures varying between about 350 pounds per square inch gauge and about 2000 pounds per square inch gauge, at a liquid hourly space velocity varying between about 0.1 and about 4, and at temperatures varying between about 650° F. and about 825° F.; the method of initiating said recycle cracking process that comprises initially contacting with said catalyst a mixture of a light gas oil

boiling within the range varying between about 390-400° F. and about 600-650° F. with said heavy gas oil in which the volumetric ratio of said light gas oil to said heavy gas oil varies between about 1:1, respectively, and about 5:1, respectively, in the presence of hydrogen and under substantially the same conditions of hydrogen to hydrocarbon molar ratio, pressure, space velocity and temperature that are employed in said recycle cracking process, continuing to charge said mixture for a period of time to produce sufficient cycle stock for said recycle cracking process, and subsequently replacing said light gas oil in said mixture of light gas oil and heavy gas oil with said cycle stock.

4. In a recycle cracking process wherein a mixture of a heavy Kuwait gas oil boiling within the range varying between about 650° F. 5 percent point in vacuum assay and about 815° F. 95 percent point vacuum assay with cycle stock boiling above about 390° F. obtained from hydrocracking said heavy gas oil and in which the volumetric ratio of said cycle stock to said heavy gas oil varies between about 1:1, respectively, and about 5:1, respectively, is contacted with a catalyst comprising between about 0.1 percent and about 5 percent, by weight of the catalyst, of platinum deposited upon a synthetic composite of silica and alumina, said composite having an activity index of at least 25, in the presence of hydrogen in amounts, expressed in molar ratio of hydrogen to hydrocarbon charge, varying between about 5 and about 50, at pressures varying between about 350 pounds per square inch gauge and about 2000 pounds per square inch gauge, at a liquid hourly space velocity varying between about 0.1 and about 4, and at temperatures varying between about 650° F. and about 825° F., the method of initiating said recycle cracking process that comprises initially contacting with said catalyst a mixture of a light Kuwait gas oil boiling within the range varying between about 400° F. and about 650° F. with said heavy gas oil in which the volumetric ratio of said light gas oil to said heavy gas oil varies between about 1:1, respectively, and about 5:1, respectively, in the presence of hydrogen and under substantially the same conditions of hydrogen to hydrocarbon molar ratio, pressure, space velocity and temperature that are employed in said recycle cracking process, continuing to charge said mixture for a period of time to produce sufficient cycle stock for said recycle cracking

process, and subsequently replacing said light gas oil in said mixture of light gas oil and heavy gas oil with said cycle stock.

5. In a recycle hydrocracking process in which a mixture of a heavy hydrocarbon charge stock and a cycle stock boiling above about 390° F. obtained from hydrocracking said heavy hydrocarbon charge stock is hydrocracked by passing said mixture at hydrocracking reaction conditions over a catalyst comprising at least one metal of the platinum and palladium series of metals, in an amount within the range about 0.05 to 20 percent, by weight of the catalyst, deposited on a synthetic composite of the solid oxides of at least two elements of groups IIA, IIIB and IV of the periodic arrangement of elements, said composite having an activity index of at least 25, the method of initiating said recycle cracking process which comprises: initially contacting said catalyst with a mixture of a light hydrocarbon charge stock boiling within the range about 390° F. to 650° F. and said heavy hydrocarbon charge stock, the volumetric ratio of said light hydrocarbon charge stock to said heavy hydrocarbon charge stock being within the range about 0.1:1 to 10:1 and hydrocracking said mixture under hydrocracking conditions which result in a net consumption of hydrogen by the mixture; continuing to charge said mixture until there is produced sufficient cycle stock to operate said process in the usual manner and then discontinuing the use of light hydrocarbon charge stock in said mixture and replacing the light hydrocarbon charge stock with cycle stock produced in the process.

6. The process of claim 5 in which, as the cycle stock is produced, it is returned to said catalyst and replaces an equivalent volume of light hydrocarbon charge stock in said mixture until said light hydrocarbon charge stock is completely replaced with cycle stock.

#### References Cited in the file of this patent

#### UNITED STATES PATENTS

|    |           |                 |       |               |
|----|-----------|-----------------|-------|---------------|
| 40 | 2,479,109 | Haensel         | ----- | Aug. 16, 1949 |
|    | 2,799,626 | Johnson et al.  | ----- | July 16, 1957 |
|    | 2,862,874 | Boedeker et al. | ----- | Dec. 2, 1958  |
| 45 | 2,885,346 | Kearby et al.   | ----- | May 5, 1959   |
|    | 2,914,461 | Ciapetta        | ----- | Nov. 24, 1959 |